

Sept. 27, 1927.

1,643,374

A. L. CLAPP

HEEL AND METHOD OF MAKING THE SAME

Filed March 7, 1924



Fig. 1.



Fig. 2.



Fig. 5.



Fig. 6.



Fig. 7.



Fig. 8.



Fig. 9.



Inventor:  
Albert L. Clapp,  
by Wright Brown Linley May,  
Atty's.

Patented Sept. 27, 1927.

1,643,374

# UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS.

## HEEL AND METHOD OF MAKING THE SAME.

Application filed March 7, 1924. Serial No. 697,489.

This invention relates to the manufacture of heels or heel bases from fibrous materials such as cellulose fiber and gums, the material being molded to form. It has heretofore been attempted to do this by filling the mold with a loose mixture of fiber and gums, waxes, resins, or asphalts and then compacting it under heat and pressure. Heels or heel bases made in this manner have not proved to be satisfactory, however, since, without an excessive amount of gums or other thermoplastic material, they are too friable and with a greater amount of gums they are brittle and relatively expensive. The friability is undoubtedly due to the fact that the fibers are not closely held together when the mass is formed up in this manner. It is also difficult to press this material together since it involves a great reduction in volume from the loose to the pressed condition.

I have discovered that these undesirable characteristics of heels or bases made of this material may be wholly overcome, and satisfactory articles produced from the same material if it is first sheeted or felted together as on a paper machine, a sufficient number of lifts died out from the sheet and assembled in superposed relation in a molding press, and then, under heat and pressure, molded to the desired shape. The lifts are condensed and fluxed together by this treatment to a sufficient extent to permit the formation of a concavity in the upper face of the heel or base to engage the heel seat of the shoe and to take clearly the size imprint from the die without the necessity of using a rand, although the extent of reduction in volume of the material is much less than when it is attempted to compress the unfelted loose mixture to final form. Not only is the strength of the article very much increased by this procedure, but its external finish is much improved, eliminating the necessity of performing any subsequent shaving operation thereon after attaching it to the shoe, buffing and polishing only being required. When formed in this manner it is also possible to employ relatively cheap fibrous material and a relatively small amount of gums, thus materially cheapening the product. It is found also that waste from the manufacture of box toe stiffeners comprising fibrous material saturated with

a thermoplastic may be used to obtain the desired thermoplastic constituents with entirely satisfactory results. A rubber heel may be readily vulcanized to the base made in this manner, if desired, or any other desired construction of top lift may be applied thereto.

For a more complete understanding of this invention, reference may be had to the accompanying drawings in which

Figure 1 is a perspective of a piece of sheet material formed on the paper machine showing lifts cut therefrom.

Figure 2 is a similar view of a lift.

Figure 3 is a perspective of a finished heel base pressed up from a plurality of lifts.

Figure 4 is an elevation of the heel press-  
ing die.

Figure 5 is a section on line 5—5 of Figure 4.

Figure 6 is a section on line 6—6 of Figure 3.

Figure 7 is an inverted plan of the upper pressure plate of the die.

Figure 8 is a section on line 8—8 of Figure 7.

The material which may be employed for constructing heels or heel bases according to this invention is susceptible of wide variation, but as one example, the furnish to be sheeted may be as follows. 60 parts of sulphate pulp, 40 parts of box toe waste, 10 parts of Montan wax, and 4 parts of red oxide, are beaten up together for approximately three hours. 5 parts of silicate of soda may then be added and beaten in for 10 minutes, and 3 parts of alum then added and beaten for 20 minutes, after which the furnish so formed is sheeted into a board of the desired caliper from which the heel lifts will be died out as will be described. In place of the sulphate pulp any other cellulose fiber, such as rags, news, or combination of any cellulose fibers, may be employed. In place of the toe waste, Montan wax may be employed or any waxes, gums, or asphalt or mixtures thereof. In place of the cellulosic materials mentioned, leather scrap may be employed.

For example, the furnish may comprise 70 parts of leather, 30 parts of toe waste, beaten together hard for 3 hours, 3 parts of silicate of soda beaten in for 10 minutes, 2 parts of rosin size beaten in for 10 minutes, and 8 parts of alum beaten in

for 20 minutes. Of course any suitable pigments for coloring the material may be employed with any of the furnishes, red oxide having been indicated in connection with the 5 furnish employing sulphate pulp.

Another furnish which has been found quite satisfactory comprises 50 parts of news; 10 parts of sulphate pulp; 5 parts of Montan wax; 35 parts of toe waste; 8 parts 10 of red oxide, beaten up together, after which 2 parts of rosin size are added and then later 3 parts of silicate of soda and then 8 parts of alum or other precipitant.

In each of the furnishes above mentioned 15 the waxes, gums, resins, or asphalts are fixed to the fibrous material by the rosin size, or silicate of soda, and the alum so that there is no difficulty in running the stock on the paper machine. The sheets thus 20 formed are air dried and preferably hot calendered so as to bring a portion of the thermo-plastic materials to the surface so that when lifts cut from this material are superposed and pressed together, the exuded 25 gums or resins tend to cause them to adhere.

The lifts 1 are cut from this sheet material shown at 2 in Figure 1 and are then placed in superposed relation within a heated mold shown at 3 in Figures 4 and 5. This mold, 30 as shown, comprises a block hollowed out to the general shape of the sides and rear of the heel or heel base, and a front plate 4 attached thereto conforming to the breast surface of the heel. The block may be 35 heated in any suitable manner as by means of electric heating units inserted at suitable openings therein, as shown at 5. The base of the mold is formed of a plunger head 6 shaped to conform to the cross section of 40 the mold, this plunger head having a stem 7 extending therefrom and projecting through an opening 8 in the block. This stem is provided for the purpose of permitting the head to be forced upwardly to eject the 45 finished heel or heel base. The die also has an upper presser head 9 having its lower face convexed and provided with size figures or other markings as 10 thereon in intaglio, 50 as shown in Figures 7 and 8. This head is also preferably heated, a resistance unit 55 11 therein being shown for this purpose.

A suitable number of lifts 1 having been placed within the mold on the head 6, the 65 heated presser head 9 is then caused to press downwardly to compress the lifts together between these heads. This pressure should be on the order of a thousand to two thousand pounds per square inch, the mold being 60 heated to a temperature of approximately 270° to 300° F. This causes the lifts to be fluxed together and condensed, the major portion of the condensation occurring at the

central portions of the lifts forming a cavity in the upper face of the finished heel 65 or base showing therein in relief sharp impressions of the insignia on the upper presser head 9. The contour of this face is suitable for engagement with the heel seat of the shoe without the necessity of cutting 70 and assembling with the lifts a separate rand strip, as is now necessary where comparatively low heels or heel bases are pressed up from laminated material of the type heretofore used. It is necessary to exert 75 this pressure in the mold for only a few seconds in order to produce the proper product.

In place of incorporating the gums, resins, or asphalts in the fibrous material before it 80 is sheeted on the paper machine, it is possible to die out lifts from sheeted fibrous material made up without these constituents, to coat them with thermoplastic material such as Montan wax, superpose them in the 85 heated mold as hereinbefore described, and subject them to pressure. In this method the Montan wax fluxes under the heat and pressure and is driven into the lifts to effect a more or less complete saturation thereof 90 so that the product is substantially the same as that produced by the other methods hereinbefore described.

Having thus described certain embodiments of this invention it should be evident to those skilled in the art that various changes and modifications might be made therein without departing from its spirit or scope as defined by the appended claims. 95

I claim:

1. The method of making heels, which comprises superposing heel lifts of felted fibrous material and thermoplastic, molding them together under heat and pressure, and vulcanizing a rubber top lift thereto. 100

2. A heel comprising superposed laminations of felted fibrous material and Montan wax fluxed and molded to form. 105

3. A heel comprising a base formed of superposed laminations of felted fibrous material and thermoplastic material fluxed and molded to form, and a rubber top lift vulcanized to said base. 110

4. A heel comprising superposed laminations of felted fibrous material containing box toe waste, said laminations being fluxed together and molded to form. 115

5. A heel comprising superposed laminations of felted fibrous material and box toe waste, said laminations containing Montan wax and being fluxed together and molded to form. 120

In testimony whereof I have affixed my signature.

ALBERT L. CLAPP.